

## UNITED STATES PATENT OFFICE

CHARLES ELLIOTT FAWKES, OF CHICAGO, ILLINOIS, ASSIGNOR TO PYROXYLIN PRODUCTS, INCORPORATED, OF CHICAGO, ILLINOIS, A CORPORATION OF ILLINOIS

## FINISHED SURFACE AND PROCESS FOR PRODUCING SAME

No Drawing.

Application filed July 9, 1928. Serial No. 291,476.

This invention relates to a new type of surface finish and a process for finishing surfaces whereby a protective coating or finish is obtained which is durable, and of unusually 5 good appearance and at a cost much below the cost of such coatings that are now in use.

Among the objects of my invention may be mentioned the finish of fibrous surfaces such as paper, imitation reed or fibre furniture, 10 wood, and the like where the material to be finished is of a porous nature, and where in many prior instances a very large part of the finishing material penetrates into the object being finished, and leaves individual fibres 15 sticking through the surface. I wish to produce in two or three coats a smooth finish on such fibrous surfaces, by applying an adhering material, glue, for example, and which material in a single coat will adhere firmly 20 without excessive penetration, and, during drying, will pull down the individual fibres and prevent their extending through the surface.

Furthermore, I desire to apply a very 25 cheap material for this purpose, preferably using water as a solvent. Another object is to have this priming coat which gives a smooth surface and excellent adherence when applied to fibrous surfaces, of such a nature 30 as to hold a subsequent finishing coat or coats firmly bound, so that there will be no danger of the bond between the final finishing coats of, for example, a lacquer enamel, and the 35 priming coat loosening and allowing the final finish to peel or otherwise loosen and separate from the glue containing coating.

The invention is especially applicable to use in finishing such surfaces as paper, wood, 40 paper fibre, and particularly fibre articles such as fibre or imitation reed furniture. The invention will be described more particularly with relation to its application in the fibre 45 furniture industry, although it will be understood that it is not limited in its application to this particular purpose.

The use of glue size for porous or fibrous surfaces is well known and has long been practiced. In finishing fibre furniture, for example, it has been customary to dip the 50 pieces of furniture in a tank of glue solution whereby the solution penetrates the fibre, carrying in some of the glue. The article is then drawn out of the tank and is allowed to drain. The water is allowed to evaporate 55 leaving a small amount of glue within the

fibre. Inasmuch as the glue solution used in the dipping tank usually contains only about 20% of glue, and the solution penetrates into the fibre, practically all of the glue size is down in the interstices, leaving the appearance of the surface practically unchanged. Furthermore, since the dipping tanks must be very large to accommodate large articles of furniture, the volume of glue solution in the tank is correspondingly large. It is necessary to hold this glue solution at temperatures above the jell point, that is, above the liquefaction point, of the glue solution. Under these conditions the glue rapidly deteriorates, and develops objectionable odors, 70 so that in a few days it becomes unfit for use and must be discarded, thus increasing the cost of the sizing process.

Even if it were possible to obtain a continuous glue film on a fibrous surface by the dipping process, it would not be possible to secure with glue alone good adherence between the glue surface and the subsequent coats of finishing material such as a lacquer or varnish.

I have discovered, however, that the addition to the glue of a substantially non-volatile substance that is soluble in both water and in the solvents used in lacquers or varnishes will render the glue surface capable of holding, 80 firmly bound, other finishing materials such as lacquer, shellac, varnish, and the like. It is, of course, necessary that the substance added to the glue be one that is compatible with both the glue and the lacquer or varnish 85 finishing coat. For example, while resorcin is soluble in both water and organic solvents such as are used in lacquers, it has a tendency to react with the glue to cause it to coagulate and it therefore is not preferable for my purpose. On the other hand, monacetin or glycerol monoacetate,



is soluble in both water and in organic solvents and is compatible with both the glue and the varnish or lacquer, and is therefore capable of producing, in a very satisfactory manner, the results which I desire to obtain, namely, a continuous coating of glue and 100 monacetin capable of forming a bond with lacquer or varnish coatings when such coatings are applied to the said continuous coating of glue and monacetin. A feature of my process, therefore, is a priming coat consist- 105 110

ing of a glue-like substance and a substantially nonvolatile material which is capable of giving to the glue-like coating the property of adhering to subsequent finishing coats such as varnish, lacquer, shellac and the like. The process of rendering glue suitable for use in the herein described process is given in detail in my co-pending application Ser. No. 251,665, filed February 3, 1928.

10 It has been previously mentioned that in processes heretofore known or practiced a very great amount of glue is required, which must be applied by a multiplicity of applications to give a continuous glue film on the 15 surface of fibrous material. Since this loads up and greatly stiffens the fibre, it is not at present the practice to use so much glue as to give a continuous film on the surface, and furthermore even if such a film were formed 20 the adherence of subsequent finishing coats would not be satisfactory.

According to the preferred form of my present invention, I apply a coating of suitable adhesive material to the surface by a hot 25 spray, preferably with steam. For example, a 30 to 40% water solution of glue containing the proper amount of monacetin as hereinbefore mentioned and heated to a temperature above the liquefaction point of the glue 30 solution is sprayed onto the surface by means of a suitable spray gun such as is used for spraying varnish or lacquer. My preferred method of applying this spray of glue is to use steam instead of compressed air to atomize the glue and monacetin solution. While 35 air that has been heated to a temperature preferably above the liquefaction point of the glue may be used, steam at a suitable pressure to give atomization has certain advantages in 40 that the particles of glue solution emitted from the spray gun do not cool down, by evaporation or otherwise, to a temperature below the liquefaction or jell point of the glue solution before they come in contact with and 45 attach themselves to the surface to be finished. By thus holding the warm glue solution at a temperature above its liquefaction point until it is deposited on the surface, a smooth continuous film of glue and monacetin 50 is obtained. It is to be understood, of course, that other suitable substances, such as sulphonated castor oil may be substituted for monacetin.

Where a glue-like film is deposited by the 55 above method, it jells very rapidly after being deposited, and, of course, the amount which "soaks in" is comparatively small. Another advantage in applying the glue-like material by a hot spray is that a comparatively thick film may be built up in one spraying 60 operation or coat. In practice it has been found that a smooth glossy finish can be obtained by one coat even on such fibrous material as blotting paper, thus giving a smooth 65 even surface for finishing with lacquer, shel-

lac, varnish and the like finishing materials.

The results that can be obtained by my process are unique in the art of finishing due to certain inherent virtues of a glue-like priming coat. This priming coat should not be confused with the ordinary glue sizing process, since a glue size is expected to penetrate the fibrous or porous material and substantially disappear from the surface. My glue priming coat, on the other hand, penetrates only a short distance into the fibre before it cools to the jell state, and permits the material to remain on the surface of the object as a continuous film, which may be of any desired thickness. Furthermore, should any fibres extend through the surface, where it is desirable to apply a relatively thin coat, the shrinkage during the drying stages of the glue jell tend to pull the fibres down so as to give a perfectly smooth surface, free from projecting fibres.

It has long been realized that if an inexpensive and proper finish could be put on paper, cloth, felt, straw and other fibrous material, such materials could be utilized to a greater extent in the fabrication of many articles. With my process, I can produce a finish on the surface of fibrous materials, such as the above, that compares favorably with the high grade finishes usually obtained on smooth metal surfaces. Thus cotton braid hats can be given a finish in two coats that gives them all of the appearance of the more expensive silk or rayon braid hats. Furthermore, when the second coat is a nitrocellulose 95 containing lacquer, the braid is rendered substantially waterproof. Straw hats can be given a glaze that has heretofore not been obtainable by any other finishing process now known. Burlap or canvas walls can be given a glossy finish by applying, by my process, one coat of my modified glue solution and one or two coats of varnish or lacquer enamel. This has not been possible heretofore, except where a great number of coats 100 of varnish is used, and where a nitrocellulose lacquer enamel finish is desired, it is necessary to use from six to eight coats in order to get a finish of an appearance that is equal 105 to the appearance that can be obtained from a coat of modified glue and one coat of lacquer according to my process. It is apparent, therefore, that my invention offers immense 110 economical advantages in the art of finishing.

The following paragraphs, denoted by numerals, indicate some of the considerations, conditions and requirements involved in connection with the present invention.

#### 1. Preparation of the glue containing composition

From 10 to 50 parts of glue is mixed with 50 to 90 parts of cold water and the glue allowed to "swell". The "swelling" consists 120 of the penetration of the water into the glue, 125

so that the mixture becomes jelly like. Depending upon the size of the glue particles and the grade of glue, this requires from 10 minutes to 2 hours. In practice, it is 5 usually preferable to allow the swelling to continue until there are no hard particles of glue remaining. The swelled glue and water mixture is then warmed up until the liquefaction point is reached, which is indicated 10 by the jell turning from a jell to a liquid state, such as is well known in preparing gelatin jells. When the glue and water have completely liquefied, there is added, for example, from one to twenty parts of a com- 15 pound such as monacetin, sulphonated castor oil, methyl or ethyl urea, and the like. If it is more convenient, the monacetin or other mutually soluble substance may be added to the water in which the glue is placed for 20 swelling. The materials which are suitable and desirable for this purpose are preferably substantially nonvolatile organic compounds which are mutually soluble in water and in organic solvents such as alcohol, butyl ace- 25 tate, turpentine and the like. Furthermore, as has already been mentioned, the material should be compatible with both glue and the materials used for subsequent coats of finish.

Where monacetin is used, it acts also as a 30 plasticizing agent for the glue, so that where a glue plasticizer is desired it may not be necessary to add any additional plasticizer. In some cases, however, it is desirable to add additional glue plasticizer, in which case any 35 of the well known glue plasticizers such as glycerin may be used. Pigments, fillers, dyes, and the like may also be added to the glue containing solution where this is desirable. Also, where it is desirable to keep the glue 40 solution for a period of time, any of the well known glue preservatives may be used. Since, according to my process, only a relatively small amount of the above described modified glue solution need be held above the 45 jell temperature during its application, the glue containing composition may be kept in cold storage over relatively long periods of time.

Various modifications are of course pos- 50 sible such as the addition of the material to the water used for swelling the glue, etc.

## 2. Application of the glue containing composition

55 As before mentioned, it is desirable to apply the glue containing composition to the surface of the article to be finished, having only sufficient penetration to give good adhesion of the glue to the material being 60 finished. My preferred method is to spray the glue composition described above at a temperature above its jell point. The glue composition is therefore held at a temperature above its temperature of liquefaction 65 and sprayed by any of the well known spray-

ing equipments such as are used for spraying lacquers, shellac, varnish, and the like.

In any case, the most satisfactory results are obtained when the temperature of the glue containing solution is held above its liquefaction point until it is finally deposited on the surface to be finished, otherwise a rough or pebbly surface may result. Although in certain types of finishes a pebbly surface may be desirable, for most purposes 75 a smooth glossy finish is the type in most general use.

In order to maintain the glue-like material at a temperature at or above its liquefaction temperature, I prefer to employ steam as a 80 medium of atomization. That is, instead of heating the glue to a very high temperature in order to compensate for the cooling effect due to evaporation of water and to the trans- 85 fer of heat from the solution to the air between the time the spray leaves the spray gun nozzle and it reaches the surface being finished, I can employ pressure steam. The use of steam will be readily apparent, as it 90 will readily be seen that the steam will not only prevent evaporation from the particles of spray by maintaining a moisture saturated atmosphere, but will give up its own heat and maintain a temperature during the whole operation above the jell point of the glue solution. 95 One of my preferred methods of applying the glue containing material is, therefore, the use of pressure steam instead of air for operating the spray gun. The source of steam may be attached to any suitable spraying apparatus at the connection ordinarily used for air. The steam pressure required 100 may be the same as the air pressure required on the spray gun to give similar atomization in the spraying of lacquers, varnishes, shellac and the like. The glue containing solution must be held at a temperature above its jell 105 temperature at the time it enters the spray nozzle. Mixtures of steam and air may be 110 used.

Under the conditions described above, the glue containing solution cools very rapidly upon striking the cold surface, and jells before it is "soaked" into the fibrous or porous material being finished. The amount of penetration can be controlled by the viscosity of the glue containing solution, the temperature of the surface being finished, the temperature at which the glue is applied, and by 120 the rate of application.

## 3. Application of final finish

Since the glue-like priming coat described above is softened by water, it is a part of my complete process to put one or more coats of a water resistant finish over the glue priming coat. I have found that a glue priming coat containing such substances as monacetin, sulphonated castor oil, and like substances, as 125 130

has already been described, enables me to secure extremely great adherence of such water resistant finishing materials as varnish or varnish enamels, nitrocellulose lacquers, shellac, and the like. These may be applied by any of the well known methods such as with a brush or with a suitable spraying equipment. It is, of course, obvious that these water resistant coatings may be of any type 10 adapted to my particular purpose, namely the protection of the glue containing priming coat against the action of water.

It is to be understood that many modifications of my invention are possible both as to 15 the choice of materials, the proportions of materials used, and the method of applying the materials to the surface being finished without departing from the spirit of the invention, or exceeding the scope of the appended claims. The herein described invention is therefore defined by the claims.

In the following claims the term "surface coating" is to be interpreted substantially as the equivalent of "protective coating", and the term "glue" as intended to include any adhesive-like material having the functions and capabilities of glue in the connection herein mentioned.

What I claim is:

30 1. A material carrying a protective coating comprising a continuous coating of glue and a substantially non-volatile glycerol ester and one or more coats of a nitrocellulose containing finishing material applied to the glue 35 containing priming coat.

2. A material carrying a protective coating comprising a continuous coating of glue and monacetin and one or more coats of a lacquer or varnish finishing material applied 40 thereto.

3. A material carrying a protective coating comprising a continuous coating of glue and monacetin and one or more coats of nitro-cellulose containing finishing material 45 applied thereto.

4. A fibrous material carrying a tightly adhering coating containing glue and a water soluble glycerol ester and one or more coats of cellulose ester containing finishing material including a vegetable oil applied thereto. 50

5. A fibrous material carrying a tightly adhering coating containing glue and a water soluble glycerol ester and one or more coats of nitrocellulose containing finishing material applied thereto. 55

6. A woven fibre body carrying a tightly adhering coating comprising a priming coat of glue and a water soluble glycerol ester and one or more coats of nitrocellulose containing 60 finishing material applied to said coating of glue and glycerol ester.

7. A fibrous surface carrying a tightly adhering coating comprising a priming coat of glue, a water soluble glycerol ester and a pigment, and one or more coats of nitrocellulose 65

containing finishing material applied to said glue containing priming coat.

8. The herein described process comprising spraying a water solution of glue and a glycerol ester to a surface as a priming coat 70 wherein steam is employed for securing atomization, allowing the glue containing coat to dry and applying thereto one or more coats of a nitrocellulose containing finishing material. 75

9. The herein described process of finishing fibre furniture, comprising applying a film containing glue and a water soluble glycerol ester wherein steam is employed to produce atomization of the glue containing 80 solution, allowing the film to dry and applying thereto one or more coats of a nitrocellulose containing finishing material.

10. The herein described process of finishing fibre furniture comprising spraying a water solution of glue and a glycerol ester and a pigment as a priming coat on the surface of said fibre furniture and wherein steam is used to secure atomization of said 85 glue containing solution, allowing the said priming coat to dry and applying thereto one or more coats of a nitrocellulose containing finishing material.

11. The herein described process of finishing absorbent surfaces comprising making a water solution of glue and a substantially non-volatile organic substance soluble in both water and organic solvents said solution having a jell point higher than the surface to which it is to be applied, heating 90 the said solution above its jell point to cause it to liquefy, applying the liquefied glue containing solution in its liquid condition under such conditions of temperature that said glue solution cools and jells before it has 95 time to be absorbed by said absorbent surface, allowing the glue containing coating to dry, and applying thereto one or more coats of a nitrocellulose base finishing material. 100

12. The herein described process comprising applying a solution of glue and a glycerol ester to a surface, allowing the glue containing coat to dry, and applying thereto one or more coats of a cellulose ester containing 115 finishing material.

13. The herein described process comprising applying a solution of glue and a glycerol ester to a surface, allowing the glue containing coat to dry, and applying thereto one or more coats of a water resistant varnish. 120

14. The herein described process comprising applying a solution of glue and a glycerol ester to a surface, allowing the glue containing coat to dry, and applying thereto one or more coats of a laquer having as a base a cellulose derivative dissolved in organic solvents. 125

15. The herein described process of finishing absorbent surfaces comprising applying on said surface a mixture of glue and glycerol

ester in water at a temperature above the jell point of the glue under such conditions of temperature that the glue containing solution cools to a jell before being wholly absorbed in the said absorbent surface, allowing the glue containing coat to dry, and applying thereto one or more coats of a lacquer including a cellulose derivative dissolved in organic solvents.

10

16. The herein described method of rendering glue capable of forming a bond with cellulose ester base lacquers, comprising adding to a glue a glycerol ester that is soluble both in water and in the solvents of the lacquer.

CHARLES ELLIOTT FAWKES.

75

15

80

20

85

25

90

30

95

35

100

40

105

45

110

50

115

60

120

125